

July 22, 1969

V. L. BULLOUGH

3,457,158

## CELL LINING SYSTEM

Filed Oct. 2, 1964



**INVENTOR**

Vaughn L. Bulloch,

BY Glenn, Palmer & Matthews

ATTORNEYS

1

3,457,158

## CELL LINING SYSTEM

Vaughn L. Bullough, Florence, Ala., assignor to Reynolds Metals Company, Richmond, Va., a corporation of Delaware

Filed Oct. 2, 1964, Ser. No. 401,067

Int. Cl. C22d 3/12, 3/02

U.S. Cl. 204—243

9 Claims

## ABSTRACT OF THE DISCLOSURE

Controlling the thermal expansion characteristic of powdered alumina by admixing therewith up to about 20% by weight of a fluoride of aluminum, such as cryolite; and electrolytic reduction cells lined with a layer of such an alumina-fluoride mixture, the expansion characteristic of which is greater than that of alumina for a fluoride content of about 10% to about 20% and less than that of alumina for a fluoride content of about 0.1% to about 5%.

This invention relates to electrolytic cells for the production of aluminum and other metals and to a novel method for controlling the thermal expansion of cell insulating materials. More particularly, the invention concerns a novel method for controlling the thermal expansion of powdered alumina.

Aluminum metal is conveniently produced in electrolytic cells by passing a current through a bath of molten cryolite containing dissolved alumina in a large tank lined with carbon which serves as one electrode, namely the cathode. Large carbon blocks presented at the top of the bath function as the anode. Molten aluminum metal at a temperature of about 1800° F. collects to the bottom of the cell and is siphoned therefrom periodically. The cells may be lined with rammed carbon and may have a row of horizontal graphite bars extending from one side of the cell which serve to contact the pad of molten aluminum which collects at the bottom of the cell when in operation, thus acting as cathode current collectors. In newer types of construction of electrolytic reduction cells, refractory linings made of alumina and cryolite are employed, as illustrated, for example, in U.S. Patent 3,093,570, and in copending application Ser. No. 222,079, now U.S. 3,321,392, filed Sept. 7, 1962. In cells of this type, current collectors extending into the aluminum metal layer of the cell are made of substances such as graphite or the borides, nitrides and carbides of elements of Groups 4, 5 and 6 of the Periodic System, particularly zirconium and titanium, for example, titanium diboride.

In the construction of aluminum reduction cells it is the practice to provide a powdered insulating layer between the cathode and the shell of the cell. The insulating powder underlies the molten metal pad and surrounds the cathode contacts, whether they be of graphite or titanium boride. When the cell is in operation a glazed layer forms on the upper surface of the insulating material, adjacent the molten metal pad, and provides a boundary between the molten metal and the bulk of the insulating powder.

Whether the cathode collectors are made of graphite or of titanium boride, it is of importance to match the thermal expansion of the insulating layer of the cell as closely as possible to the thermal expansion of the cathode collector in order to minimize thermal stresses which may tend to produce failure of the cathode collectors.

It has been found that the thermal expansion characteristics of the cell insulation material can be tailored to correspond closely with those of the cathode collector material. This is accomplished, in accordance with the invention, by incorporating in the powdered alumina used

2

for the cell insulating material a minor proportion of a fluoride of aluminum.

The fluoride of aluminum may be aluminum fluoride,  $AlF_3$ , or it may be a double fluoride of aluminum and an alkali metal, such as cryolite  $NaF \cdot AlF_3$ . These fluorides are intimately admixed with powdered alumina in a proportion ranging from about 0.1% to about 20% by weight. In proportion to the amount of fluoride added, it has been found, surprisingly and unexpectedly, that the thermal expansion of the powdered alumina may be controlled, with the result that it may be either diminished or increased. Thus, for example, the addition of from about 0.1% to about 5% of cryolite by weight to alumina powder brings about a decreased thermal expansion, whereas the addition of from 10% to 20% produces an increase in thermal expansion.

The effect of additions of cryolite to alumina in diminishing or increasing its linear thermal expansion may be seen from the curves of the accompanying drawing. The relationship of linear expansion to temperature for pure alumina is shown in the broken line curve. The addition of 5% of cryolite is reflected in the group of curves lying below the pure alumina curve, while the addition of larger amounts of cryolite elevates the thermal expansion curve. The curves of the drawing are based upon experimental data obtained by measuring thermal expansion of compacted alumina powder at temperatures to 1000° C. in a silica dilatometer. The dilatometer was constructed by modifying a porcelain filter crucible (Selas No. 6010) by installation of a thermocouple well through its bottom and extending into the crucible approximately one inch, the well being cemented into place. The powdered material to be tested for thermal expansion was placed in the test crucible and packed by tapping the bottom. The crucible containing the sample was placed within the cavity of a wire-wound silica dilatometer furnace and heated to 1000° C. at the rate of about 2.8° C. per minute. The linear expansion of the sample was measured to the nearest 0.0001 inch by means of a dial indicator, the expansion being transferred to the dial by means of a fused silica rod placed on top of the sample within the dilatometer furnace.

In accordance with the novel method of the invention, the admixing of the fluoride with the alumina powder is performed in any suitable type of mixing apparatus, the mixing being carried on until a uniform mixture is obtained.

The practice of the invention is illustrated by the following example, which is not, however, to be regarded as limiting:

## Example

Where an aluminum reduction cell is constructed so as to include bottom entry graphite cathode collectors, in the manner illustrated, for example, in FIG. 6 of Patent 3,093,570, the thermal expansion of the alumina insulating layer may be controlled to match that of the graphite, which is substantially less than for powdered alumina. The mean temperatures of the graphite and the alumina lining will depend upon the cell design. However, the thermal conductivity of the graphite is about 1000 times that of the powdered alumina. In practice, the graphite temperature is about 900° C. A reasonable mean temperature for the alumina may be assumed to be about 550° C. The junction of the glazed layer previously mentioned and the graphite collector is below the top of the graphite collector, the relative position depending upon the design and operation of the cell. The longitudinal thermal expansion of graphite at 900° C. is about 0.3% (Carbon Products Handbook p. 19, 1964 Ed., Union Carbide Corp., New York). Assuming that about 75% of the graphite member is embedded in the alumina layer, the

problem is one of employing a refractory mixture that has the same average thermal expansion at 550° C. over its length as the graphite member has over its length, i.e. about 0.225%.

In accordance with the present invention, it has been found that a mixture of 99% alumina and 1% cryolite has an expansion coefficient of 0.21%. Thus, for the design in question, a mixture of 99 parts by weight alumina to 1 part by weight of cryolite will prevent tension stresses in the graphite, providing an expansion of the alumina powder which is compatible with the graphite collector.

Employing similar considerations, the thermal expansion of the alumina insulating layer may be controlled to match that of a titanium diboride cathode collector.

There may also be employed a suitable mixture of powdered alumina and aluminum fluoride as a bed material for a reduction cell.

It will be appreciated, furthermore, that the insulating or bed layer may be subdivided into two or more layers, each adjusted by addition of cryolite or aluminum fluoride so as to provide suitable expansion characteristics for a particular area.

What is claimed is:

1. An electrolytic reduction cell having an interior lining consisting essentially of a powdered mixture of alumina and from about 0.1% to about 20% by weight of a fluoride of aluminum, with a conductive cathode extending at least partially therethrough for contact with the molten contents of the cell, said lining having a thermal expansion substantially similar to that of said cathode.

2. An electrolytic reduction cell having an interior lining consisting essentially of a powdered mixture of alumina and from about 0.1% to about 5% by weight of cryolite, with a graphite cathode extending at least partially therethrough, said lining having a thermal expansion substantially similar to that of said graphite cathode.

3. An electrolytic reduction cell having an interior lin-

ing consisting essentially of a powdered mixture of alumina and from about 10% to about 20% by weight of cryolite, with a titanium diboride cathode extending at least partially therethrough, said lining having a thermal expansion substantially similar to that of said titanium diboride cathode.

4. The cell of claim 1 in which the fluoride of aluminum is cryolite.

5. The cell of claim 1 in which the fluoride of aluminum is aluminum trifluoride.

6. Method of lining an electrolytic reduction cell, which consists essentially of intimately admixing powdered alumina with from about 0.1% to about 20% by weight of a fluoride of aluminum and then tamping said powdered mixture into the bottom of the cell so that a cathode of conductive material extends at least partially therethrough, said mixture having a thermal expansion substantially similar to that of said conductive material.

7. The method of claim 6 in which the conductive cathode material is graphite.

8. The method of claim 6 in which the conductive cathode material is titanium diboride.

9. The method of claim 6 in which the fluoride of aluminum is cryolite.

#### References Cited

##### UNITED STATES PATENTS

|           |        |          |       |         |
|-----------|--------|----------|-------|---------|
| 3,028,324 | 4/1962 | Ransley  | ----- | 204—243 |
| 3,093,570 | 6/1963 | Dewey    | ----- | 204—243 |
| 3,261,699 | 7/1966 | Henry    | ----- | 204—243 |
| 3,267,183 | 8/1966 | Feinleib | ----- | 204—243 |

JOHN H. MACK, Primary Examiner

D. R. VALENTINE, Assistant Examiner

U.S. Cl. X.R.

204—67; 264—30